

Oct. 27, 1936.

J. N. OSTROFSKY

2,058,494

PRODUCTION OF FERRO ALLOY

Original Filed July 20, 1933



Inventor:  
James N. Ostrofsky,  
By John Howard Joynt,  
his Atty.

## UNITED STATES PATENT OFFICE

2,058,494

## PRODUCTION OF FERRO-ALLOY

James N. Ostrofsky, Baltimore, Md., assignor, by  
mesne assignments, to Rustless Iron and Steel  
Corporation of America, Baltimore, Md., a cor-  
poration of Delaware

Original application July 20, 1933, Serial No.  
681,371. Divided and this application October  
27, 1933, Serial No. 695,549

6 Claims. (Cl. 75—11)

This invention is divided out from my co-pending application Serial Number 681,371, filed July 20, 1933, entitled Ferro-alloy and relates to ferro-alloys, more particularly to iron-chromium 5 alloys, and to an art of producing the same.

One of the objects of my invention is the production of an iron-chromium alloy of high chromium and nitrogen contents which readily lends itself to an ease of handling and wide 10 range of application in the production of rust-less iron and steel.

Another object is the production of a high grade alloy of the class indicated in a simple, reliable, and thoroughly practical manner at 15 maximum efficiency and minimum expense.

Another object is the direct and economical production of a nitrogen containing iron-chromium alloy of high nitrogen and chromium contents employing known furnacing equipment 20 and handling apparatus.

Other objects will be obvious, in part, and in part pointed out hereinafter.

The invention, accordingly, consists in the features of construction, combination of elements and arrangement of parts, and in the several steps and the relation of each of the same to one or more of the others as described herein and the scope of the application of which is indicated in the following claims.

30 In the single figure of the accompanying drawing there is illustrated, in vertical section, electric furnace apparatus for carrying out the practice of my invention.

Referring now more particularly to the practice of my invention, a suitable electric furnace, (see the accompanying drawing) for example, a 2-ton single-phase electric arc furnace, rated 60 cycle, 200 kw. at 110-180 volts, and having two carbon electrodes projecting downwardly into 40 a magnesite lined furnace shell is prepared for the reception of a charge of raw materials. Conveniently an open-top furnace having a metal shell 10, a magnesite lining 11 and electrodes 12 and 13 is used, although it will be understood that a furnace having a lid which gives an enclosed furnace chamber may be employed where desired. As a matter of convenience the furnace is mounted on a suitable foundation 14 to permit the furnace tap-hole 15 being positioned at a convenient height above the floor of the melt-shop. The furnace electrodes are supported in any suitable manner, not shown, to permit desired adjustment.

Power is supplied the furnace from an electrical transformer (not shown), with voltage

control apparatus, connected to a suitable source of electrical energy. Conveniently, electrical energy is applied to the furnace electrodes 12 and 13 respectively by flexible cables 16 and 17 connected to desired transformer and control 5 apparatus.

In preparing the furnace for the reception of a charge of raw materials, power is applied and an arc struck from the furnace electrodes to a small amount of crushed ferrochrome strung 10 along the furnace bottom between the projected electrodes. When the furnace bottom and side walls are thoroughly heated, chrome ore together with a suitable reducing agent, such as coke, and desired fluxing agents, lime and fluorspar, 15 are added as rapidly as furnace conditions permit. The proportion of the charge first added melts down under the action of the intense heat of the electric furnace arcs to form a slag containing the oxides of iron and chromium which 20 overlies the small pool of metal on the furnace bottom. The reducing agent added along with the initial charge of ingredients is in part distributed throughout the slag and serves to effect a reduction of the oxides of iron and chromium. 25 The reduced metals gravitate through the slag into the underlying pool of metal formed upon the furnace bottom.

In order to achieve an iron-chromium alloy of high nitrogen content, an inexpensive nitrogen 30 containing gas such as ammonia, is preferably directly introduced into the slag during the reduction of the oxides of iron and chromium contained therein. The ammonia gas readily dissociates into the component gases hydrogen and 35 nitrogen. While the former gas, in a manner, serves as a reducing agent to aid in the reduction of the reducible oxide content of the slag, and so permit a decrease in the amount of the reducing agent employed, the latter gas is ac- 40 tively absorbed by the nascent iron and chromium formed during the reduction of the oxides of these metals contained in the slag. This nitrogen is then carried into the metal beneath the slag. The incidental absorption of hydrogen 45 gas by the nascent metals is, in most instances, unobjectionable in the production of ferro-alloys of the class indicated. Best results in the production of a ferrochrome of high nitrogen content is achieved by introducing nitrogen containing gas directly into those regions of the slag where the reduction of the oxides is most ac- 50 tively going on. Ordinarily this is within the regions adjacent the furnace electrodes.

With the continued application of power and 55

further introduction of the raw materials, chrome ore, coke, lime and fluorspar into the furnace, more and more of the molten metal containing iron, chromium and nitrogen is formed. This metal may be tapped out of the furnace through a suitable tap hole in the furnace wall adjacent the bottom while further operation of the furnace continues, or the furnace may be tapped after the preparation of a heat of metal is substantially complete and the slag covering the metal is removed.

As illustrative of the practice of my invention, 12,000 pounds of chrome ore analyzing about 51.4% chromium oxide ( $\text{Cr}_2\text{O}_3$ ), 16.7% iron oxide ( $\text{FeO}$ ) and with the balance oxides of aluminum, magnesium, and silicon, is charged into a furnace of the character illustratively indicated above which is previously prepared for the reception of the charge. Along with the chrome ore there is charged 3600 pounds of coke, together with 125 pounds of lime and 300 pounds of fluorspar. These ingredients are preferably mixed prior to charging into the furnace so that the reducing agent, coke, and the fluxing agents, lime and fluorspar, are distributed throughout the charge of chrome ore. The entire charge of ingredients is added in several batches, one batch following another as rapidly as furnace conditions permit.

Under the action of the intense heat of the electric arc, (see the accompanying drawing) the first batch of ore, reducing agent, and flux commences generally indicated at 18 to fuse and forms a slag denoted 19 containing oxides of iron and chromium through which is distributed the carbonaceous reducing agent. As the ingredients fuse and become fluid, a reaction takes place between the reducing agent and the oxides of iron and chromium contained in the slag 19. These oxides are reduced and the metals formed thereby gravitate toward the bottom of the furnace forming thereon a bath of metal 20 while the gases formed as a result of this reaction escape upward, through the ingredients in the furnace, and then into the atmosphere.

Additions of the remaining batches of raw materials are made as permitted by the impoverishment of the slag through the reduction of the reducible oxide constituents thereof, as more particularly indicated above, and the complete or partial removal of this impoverished slag.

An iron-chromium alloy of desired nitrogen content is achieved as indicated above, by directly introducing a nitrogen containing gas, such as ammonia, into those portions of the slag where the reduction of the oxides of iron and chromium are taking place. For example, a gentle flow of ammonia gas is directly introduced into the slag adjacent the lowermost portions of the furnace electrodes through one or more refractory pipes 55 throughout the entire process or any part thereof as desired. For the illustrative embodiment set forth above good results are achieved by introducing ammonia gas from a suitable source (not shown) through a flexible tube 21 and a refractory pipe 22, having an inner diameter of about  $1\frac{1}{2}$ ', positioned between electrodes 12 and 13 and extending beneath the bottom level of slag 19. Pipe 22 is maintained in proper position for example, by means of parallel spaced angle irons 23 and 24 resting on the top of the furnace shell 10 and engaging an adjustable collar 25 secured to the pipe. The lower end of the refractory pipe is conveniently provided with a number of small openings 22a to permit escape of the nitrogen-containing gas out into the surrounding slag.

Preferably, the introduction of ammonia is continued throughout the entire period of the process.

The nascent iron and chromium formed during the reduction of the chrome ore absorb the nitrogen and in a measure directly combine therewith to form nitrides of iron and chromium. When substantially all of the metal is recovered from the reducible oxides contained in the chrome ore charged into the furnace (as evidenced by the appearance of the slag), the heat of metal is tapped and allowed to cool after which the metal is crushed to a desired lump size ready for shipment and use. The heat of metal weighs 5,300 pounds and analyzes approximately 59% chromium, 5% carbon, 2% nitrogen, with the balance principally iron. The metal is hard and brittle, which, when crushed, lends itself to an ease of handling and furnacing in the production of, for example, rustless irons and steels of desired nitrogen contents, the proportions of which are directly controlled.

Thus it will be seen that there has been provided in this invention a ferro-alloy of high nitrogen content and an art of producing the same in which the various objects hereinbefore noted together with many thoroughly practical advantages are successfully achieved. It will be seen that the process lends itself to the production of inexpensive nitrogen containing iron-chromium alloys of desired nitrogen content which may be controlled within commercial limits.

While, for purposes of illustration, a nitrogen containing ferrochrome of high nitrogen content is obtained it will be understood that by limiting the flow of the nitrogen containing gas into the molten ingredients during the reduction thereof, either in quantity per unit time (as by decreasing the pressure or by employing a smaller pipe) or for the total time during which nitrogen is introduced into the slag, the nitrogen content of the tapped metal may be decreased to 1 per cent or even lower (0.5% for example) as desired. So, also, by increasing the flow of nitrogen into the slag and distributing this nitrogen containing gas so as to effect a more intimate association between the gas and the nascent metals as by directing a plurality of streams of nitrogen containing gas into those regions of the slag where the reduction of the reducible oxide is most active, the nitrogen content of the tapped metal may be increased considerably even to a value approaching 15% corresponding to a complete conversion of the chromium oxide to chromium nitride ( $\text{CrN}$ ).

The proportion of chromium and iron vary in accordance with the proportions of these ingredients found in the particular chrome ore employed. For example, the chromium content of the metal may vary between about 50% and 72% depending upon the raw materials used although, ordinarily, the chromium content varies between 55% and 69%. The carbon content largely depends upon the amount of carbon in the mix (this is usually in excess of the chemically equivalent amount required to achieve a reasonably high recovery of metal from the ores) and to a lesser extent upon the type and condition of the furnace employed as well as upon the rapidity with which the process is carried out; a rapid practice of the process keeping the carbon containing atmosphere in contact with the metal a minimum length of time. By the exercise of particular care the amount of carbon may be brought as low as 1% although the carbon content ordinarily amounts to about 5%.

While in the embodiment of my invention illustratively set forth above a nitrogen containing gas is directly introduced into the slag containing the oxides of iron and chromium, and preferably 5 into those regions of the slag where the reduction of these oxides is most active, good results are achieved where the reduction of the metallic oxides is carried out in an enveloping atmosphere of nitrogen containing gas.

10 Likewise while the introduction of ammonia gas gives excellent results and permits the production of an iron-chromium alloy, the nitrogen content of which is readily controllable within commercial limits, good results are achieved 15 where nitrogen gas is employed, as from commercial bottled nitrogen.

As many possible embodiments may be made of my invention and as many changes in the embodiment hereinbefore set forth it will be understood that all matter described herein is to be interpreted as illustrative, and not in a limiting sense.

I claim:

1. In the production of an iron-chromium alloy 25 of high nitrogen content, the art which includes, reducing chrome ore, in the immediate presence of a nitrogen containing gas bubbling into and through the region undergoing reduction.
2. In the production of an iron-chromium alloy 30 of high nitrogen content, the art which includes, reducing chrome ore in the presence of ammonia gas under pressure.
3. In the production of an iron-chromium alloy 35 of high nitrogen content, the art which includes, reducing chrome ore with a suitable reducing agent and passing nitrogen gas into and through

the ore undergoing reduction whereby nitrogen is absorbed by the metals formed thereby.

4. In the production of an iron-chromium alloy of high nitrogen content, the art which includes, melting down chrome ore and a 5 reducing agent in a suitable furnace to form a slag containing oxides of iron and chromium which are reduced by said agent forming thereby the metals iron and chromium, and bubbling nitrogen gas through said slag during the reduction of the oxides contained therein whereby nitrogen is absorbed by and combines with the metals resulting therefrom.

5. In the production of an iron-chromium alloy of high nitrogen content, the art which includes, 15 continuously melting down chrome ore in the presence of a carbon reducing agent to form a slag containing oxides of iron and chromium which are reduced by said agent thereby giving nascent iron and chromium, and passing 20 ammonia into said slag during the reduction of the oxides contained therein whereby nitrogen is absorbed by said nascent metals.

6. In the production of an iron-chromium alloy of high nitrogen content, the art which includes, 25 melting down chrome ore in an electric arc furnace having carbon electrodes to form a slag containing the oxides of iron and chromium, reducing the oxides contained in said slag by a suitable reducing agent, and passing nitrogen containing 30 gas into said slag adjacent said furnace electrodes whereby nitrogen gas is absorbed by the metals resulting from the reduction of the oxides contained in said slag.

35

JAMES N. OSTROFSKY.